

April 27, 1937.

M. HAGEDORN ET AL

2,078,535

MANUFACTURE OF RELIEF PRINTING FORMS

Filed Aug. 16, 1933



Inventors:

Max Hagedorn,

Gerhard von Kujawa

Potter, Pierce & Scheffler.

By Attorneys

## UNITED STATES PATENT OFFICE

2,078,535

## MANUFACTURE OF RELIEF PRINTING FORMS

Max Hagedorn and Gerhard von Kujawa, Dessau  
in Anhalt, Germany, assignors to I. G. Farben-  
industrie Aktiengesellschaft, Frankfort - on-  
the-Main, Germany, a corporation of Germany

Application August 16, 1933, Serial No. 685,454  
In Germany August 20, 1932

3 Claims. (Cl. 101—395)

Our present invention relates to the manufacture of forms for letterpress printing.

One of its objects is a process of manufacturing forms for letterpress printing. Another object is the forms for letterpress printing. Further objects will be seen from the detailed specification following hereafter.

It has been proposed, in making relief printing forms, to impress a plastic mass with a relief 10 on a level surface, for instance, a wash-out relief produced on a chromated gelatin layer or a wash-out relief produced in a non-photographic way. When solidified, the impressed mass represents a negative of the required relief and may, 15 if necessary, be directly used as a relief printing form, after fixing it to a suitable support. This process, however, could not hitherto obtain practical importance for lack of a suitable plastic material.

According to this invention relief printing forms are made by impressing the relief serving as a pattern either in a dry or slightly wet state, 20 into a sheet or foil made of a polymerization product of an unsaturated organic compound, or of a condensation product of such a polymerization product with an aldehyde, a ketone or the like. Instead of the sheet of foil the unshaped mass of the same product may be used. The product may be a polyacrylic acid derivative 25 (such as an ester, a nitrile or a salt), a polyvinyl halide, a polyvinyl acetate, polystyrol or a mixed polymerization product, for instance, the polymerization product from a mixture of styrol and an acrylic acid ester, from a mixture 30 of a mixture of an acrylic acid ester and acrylic acid nitrile, from a mixture of styrol and a maleic acid ester, or a mixture from vinylmethyl-ether and a methylene maleic acid ester, or a condensation product, for instance, a condensa- 35 tion product from polyvinylalcohol and butyraldehyde or the like. The sheets or foils are prepared in known manner by the pressing process, the spraying process or the celluloid process, or by dissolving the product in an organic solvent 40 and producing the sheet in the desired thickness by means of a film casting machine. If required the sheet may contain an addition of softening agents, pigments, dyestuffs, filling agents and the like, known in the manufacture of plastic masses. 45 Additions of other highly polymeric substances, such as polyglycols, albuminous substances or cellulose esters, mixed cellulose esters, mixed cellulose ether esters and ethers are also possible. 50

Sheets made of polyvinyl chloride which con- 55 tains more than one halogen atom and less than

two halogen atoms on one vinyl group corresponding with the formula  $\text{CH}_2:\text{CH}_2$  have proved specially suitable for the purpose in question. Such after-chlorinated polyvinyl halides are obtainable according to the co-pending application Ser. No. 670,213, filed by Kurt Schönburg. 5

The foils have a thickness from about 0.05 to 0.1 mm. and upwards as required. Either prior to or after impression, they may be fastened to any suitable level support of metal, or the like 10 by means of a suitable adhesive substance.

The following examples illustrate the invention:

*Example 1.*—A gelatin layer applied on a level surface of metal, glass or film, sensitized with 15 potassium bichromate, is exposed under a negative for line and half-tone work and developed into a wash-out relief. This relief, while on a plane metal plate is brought into a hydraulic press and is pressed while in a dry or slightly 20 wet condition, into a foil made of polyvinyl chloride the chlorine content of which amounts to 65%. The foil is also supported on a plane metal plate and the temperature and the pressure of operation are 80 to 85° C. and 100 to 120 atmospheres, respectively. In order that the foil 25 of polyvinyl chloride may be easily detached from the gelatin relief, the latter, prior to pressing, may be treated with a solution of paraffin wax.

Instead of a relief produced from a bichromated 30 gelatin layer, a gelatin relief that has been produced in a silver halide emulsion layer by a hardening development may be used.

Instead of using the polymerization product in 35 the form of a thin foil mounted on a metal, or wooden or similar plate, it may be used in the form of a block which possesses the height necessary for the finished printing block.

*Example 2.*—A gelatin wash-out relief produced as described in Example 1 is impressed 40 in the manner described in that example into a foil made of a mixed polymerization product from vinyl chloride and acrylic acid methylester in the proportion of 3:1 at a pressure of 150 atmospheres and a temperature between 70 and 45 80° C. the duration of pressure being 5 minutes.

In the single figure of the accompanying drawing there is shown the section of a relief printing form made of polyvinyl chloride containing about 65 per cent of chlorine.

The masses used according to this invention have the advantage that they can be easily worked inasmuch as they become plastic at a temperature below 120° C., most of the compounds enumerated can even be worked at a 50 55

temperature between 70 and 100° C. Furthermore the plastic masses according to this invention can be used again. Thus the costs for the production of relief printing forms are reduced.

5 What we claim is:

1. A relief printing form comprising the polymerization product of a vinyl compound.
2. A relief printing form comprising poly-

vinyl chloride containing about 65 per cent of chlorine.

3. A relief printing form comprising the polymerization product from a mixture of vinyl chloride and acrylic acid methylester.

5

MAX HAGEDORN.  
GERHARD V. KUJAWA.